

Patented Nov. 28, 1944

**2,363,512**

UNITED STATES PATENT OFFICE

**2,363,512**

## COMPOUNDED OIL.

Bruce B. Farrington and James O. Clayton, Berkeley, and Dorr H. Etzler, Albany, Calif., as-  
signors to Standard Oil Company of California,  
San Francisco, Calif., a corporation of Dela-  
ware

**No Drawing. Application September 15, 1942,  
Serial No. 458,453**

**19 Claims. (Cl. 252—39)**

This invention relates to the improvement of hydrocarbon oils and the like, in particular, mineral lubricating oils.

This application is a continuation-in-part of our co-pending application Serial No. 322,946, filed March 8, 1940.

Hydrocarbon oils undergo deterioration during use or exposure to the atmosphere. Mere exposure to the air at relatively low temperatures, as in the case of transformer oils and switch oils, results in the gradual formation of acidic oxidation products and the deposition of sludge. Use of a lubricating oil in the ordinary gasoline engine, as in motor cars, results in a more rapid deterioration of the oil with deposition of sludge and the formation of "varnish" on cylinder walls. Use of a lubricating oil in Diesel engines, which operate at higher temperatures and pressures than ordinary gasoline engines, results in even more rapid deterioration with resultant greater disadvantages. The temperatures and pressures involved in Diesel engine operation, around 400°-650° F. and 750-1200 pounds per square inch, cause deposition, from ordinary lubricating oils on the moving parts of the engine, such as pistons, piston rings and piston ring slots, of carbonaceous matter of such a cementitious character as to cause sticking of piston rings and greatly to reduce the efficiency of the engine.

It has been found heretofore that some improvement of hydrocarbon oils, especially lubricating oils, can be effected by incorporating therein a small amount of a soap of a fatty acid, such as a sodium, calcium or magnesium soap of butyric, capric, palmitic, stearic or oleic acid. Such soaps, among other things, reduce piston ring sticking in internal combustion engines, especially Diesel engines, apparently by loosening the cementitious deposits described above, or by inhibiting the formation of such deposits, or both. The action of the added soaps, by virtue of the analogy to the common cleansing or detergent action of soaps, came to be known as a "detergent" action and the soap additives came to be known as "detergents".

The use of these soaps or detergents is not, however, without disadvantage. Among other things they are corrosive to certain alloy bearings, such as copper-lead and cadmium-silver alloy bearings, which are commonly used in internal combustion engines. So destructive are certain of the soaps to these alloy bearings that they cannot be used satisfactorily in lubricating oils for internal combustion engines.

It is an object achieved by the present invention to provide a valuable class of additives for

lubricating oils, transformer and switch oils, and the like.

It is a further object achieved by the present invention to improve the use of soap-like or metal alkyl carboxylate additives in viscous hydrocarbon oils.

It is a still further and a particular object achieved by the present invention to provide a class of soap-like or metal alkyl carboxylate additives for lubricating oils which are noncorrosive, or substantially less corrosive than prior soap additives, such as calcium stearate, toward alloy bearings.

Other objects achieved by the invention will be apparent from the description and the claims.

We have discovered that substantial advantages result from incorporating in a hydrocarbon oil or the like, especially, a hydrocarbon lubricating oil, a polar substituted metal alkyl carboxylate 20 wherein the polar substituent is of a certain class and is in an alpha, beta or gamma position with respect to a metal alkyl carboxylate group.

The substituents that have been found to be desirable are those which contain a metal or metalloid and oxygen or sulfur; that is, we add to and use in hydrocarbon oils or the like alpha, beta or gamma substituted metal alkyl carboxylates, the alpha, beta or gamma substituent being a metal- or metalloid- and oxygen- or sulfur-containing radical. Preferably, those substituents are used wherein a metal, metalloid, oxygen or sulfur atom is directly bonded to the alkyl group of the metal alkyl carboxylate.

The additives of our invention may also be characterized by the following formulae:



wherein M is a metal (or the hydrogen equivalent of a polyvalent metal), the carbon atoms shown attached to COOM are aliphatic carbon atoms, and X is a substituent containing a metal or metalloid and sulfur or oxygen. The unsatisfied carbon valencies shown may be satisfied by hydrogen or hydrocarbon groups (e. g. alkyl groups), by polar groups (including polar groups of the type represented by X, and/or other polar groups), etc.

It will be apparent that three principal constitutional factors may be varied in the additives of this invention: (1) the nature and amount of the substituent X; (2) the nature of the alkyl carboxylic acid which is substituted and whose salt is formed; and (3) the nature of the metal M. These factors are discussed in more detail immediately below.

(1) *The substituent X*

Substituents comprising oxygen or sulfur or both and at least one of the following metals and metalloids are illustrative: sodium, potassium, magnesium, calcium, barium, zinc, cadmium, aluminum, silicon, lead, arsenic, antimony, bismuth, chromium, selenium, tellurium, iron, cobalt and nickel. The metallo-carboxy and metallo-thiocarboxy groups constitute an important class of substituents within the scope of the invention; that is, the groups COOM, COSM, CSOM and CSSM, where M is the hydrogen equivalent of a metal. Other typical examples of the substituent X are as follows:



In the above, M represents the hydrogen equivalent of a metal or metalloid, such as the metals and metalloids specifically enumerated above.

Those substituents are preferred which do not hydrolyze readily to produce corrosive acids. However, insofar as certain of the advantages of the metal alkyl carboxylates of the invention are concerned, even those polar substituents which hydrolyze readily to produce corrosive acids are effective; for example, as long as the hydrolyzable polar group remains attached to the metal alkyl carboxylate, it inhibits corrosion.

(2) *The alkyl carboxylic acid*

For simplicity's sake, reference is made to the free, unsubstituted acids, and it is to be understood that in the practice of the invention a substituent will be included and a metal salt formed, as indicated hereinabove.

Mono- and polybasic acids may be employed, and although open chain acids are preferred, cycloaliphatic acids and aliphatic acids having an aromatic substituent in the alkyl chain (preferably removed by three or more carbon atoms from the alkyl carboxyl group) are comprehended by the invention. In all cases, however, the acid contains at least one carboxyl group attached to one alkyl or aliphatic carbon atom. By the term "alkyl carboxylic acid" is meant a carboxylic acid in which a COOH group is attached to an aliphatic carbon atom, and by

the term "metal alkyl carboxylate" is meant the metal salt of such an acid.

Illustrative of suitable acids are the following:

5 *Acids of the acetic series*, such as propionic, butyric, isobutyric, valeric, isovaleric, alpha-methylbutyric, pivalic, caproic; alpha, alpha-dimethylbutyric; alpha, beta-dimethylbutyric, alpha-ethylbutyric; alpha-ethyl, alpha-methylbutyric, capric, lauric, myristic, palmitic, stearic, etc.; also, unsaturated and/or hydroxy and other substituted members of the same series such as oleic, linoleic, linolenic, licanic, lactic and ricinoleic acids.

10 *Acids of the oxalic acid series*, such as malic, succinic, isosuccinic, glutaric, adipic, etc.; also, unsaturated dibasic acids, such as malic and fumaric; also, hydroxy dibasic acids, such as malic, mucic and tartaric.

15 *Tribasic acids*, such as citric and agaric acids. Preference is given to those acids, generally the longer chain alkyl carboxylic acids, whose salts are oil soluble, although the lower acids, even acetic, when properly substituted and used 20 in the form of appropriate metal salts, greatly improve the stability of hydrocarbon oils and inhibit ring sticking and associated phenomena. C<sub>10</sub> and higher acids provide adequate oil solubility.

25 (3) *The metal M*

Any mono- or polyvalent metal capable of forming a sufficiently stable salt with the acid chosen may be used. Metals which do not exhibit adverse catalytic activity (such as promoting oxidation) and whose use does not result in excessive wear are preferred. Examples of metals whose salts may be formed and used in accordance with this invention are lithium, 30 sodium, potassium, calcium, barium, strontium, beryllium, magnesium, aluminum, zinc, cadmium, tin, lead, chromium, molybdenum, tungsten, manganese, iron, cobalt, nickel, vanadium and bismuth. Basic and mixed, as well as normal simple salts may be employed. The metal of the COOM group and the metal of the X substituent may be the same, as in barium beta-phosphonato-isobutyrate



or the metal of the COOM group and the metal or metalloid of the X substituent may differ, as in calcium alpha-borylbutyrate



Examples of substituted metal alkyl carboxylates contemplated by this invention are sodium, potassium, calcium, barium, aluminum, magnesium, zinc and nickel alpha, beta and gamma metallo- (e. g. calcium, barium, or magnesium) phosphonato butyrate; the corresponding alpha, beta and gamma metallo-phosphonato valerates, caproates, caprates, laurates, myristates, palmitates, stearates, acrylates, crotonates, angelicates, oleates, lactates, malonates, succinates, glutarates, adipates, maleates, fumarates, malates, and citrates; also the corresponding metallo-thiosulfato, silicate, metallo-carboxy, metallo-thiocarboxy, metallo-thiophosphonato, seleninyl, selenonyl and boryl substituted salts (that is, the salts formed by substituting metallo-thiosulfato, silicate, etc. for metallo-phosphonato).

Highly useful additives may be produced for use in accordance with the invention by introducing a long chain alkyl group into the molecule of an aliphatic polybasic acid and forming a salt of the alkyl substituted polybasic acid, which salt has at least two metallo-carboxyl groups. This may be accomplished in several ways; for example, as follows:

1. One carboxyl of a tribasic acid such as citric acid may be esterified to produce a di-acid ester of the acid and a long chain alcohol, and the remaining unesterified carboxyls are saponified.

2. A long chain alkyl group is substituted in a



group of a polybasic aliphatic carboxylic acid.

Examples of alkyl substituted aliphatic poly-metallocarboxylates are the normal sodium, potassium, magnesium, calcium and barium and the basic aluminum salts of mono-decyl, mono-lauryl, mono-tetradecyl, mono-cetyl, mono-octadecyl and mono-eicosyl citrates; the normal sodium, potassium, magnesium, calcium and barium and the basic aluminum salts of alpha-decyl, alpha-lauryl, alpha-tetradecyl, alpha-tetradecenyl, alpha-cetyl, alpha-cetetyl, alpha-octadecyl and alpha-eicosyl tartrates, malonates, succinates and glutarates.

It will be apparent to one skilled in the art that all of the possible substituents  $X$  cannot be introduced into each of the positions alpha, beta and gamma of every alkyl carboxylic acid. Thus the presence in an alkyl carboxylic acid of an alpha, beta or gamma substituent, for example an hydroxyl substituent, may hinder the further substitution of the alpha, beta or gamma position by a certain substituent  $X$  of the present invention. In such case, a different substituent  $X$  within the scope of the invention, or a different position in the alkyl carboxylic acid, or a different alkyl carboxylic acid may be chosen for substitution; or the hindering alpha, beta or gamma group, such as an hydroxyl group, may be replaced by the desired substituent.

Various methods of forming the metal salts may be employed, one such method being to form an alkali metal salt (as by neutralizing the acid, or saponifying the corresponding ester, with an alkali metal hydroxide) and using the alkali metal salt per se or converting it into a polyvalent metal salt by adding to an aqueous solution of the alkali metal salt, a water soluble salt of a polyvalent metal, thus producing double decomposition and precipitation of the polyvalent metal salt.

The substituted metal alkyl carboxylates of this invention improve hydrocarbon oils in several respects. One of the most important improvements resulting from the use of these car-

boxylates in mineral oil lubricants is their marked detergent effect, unaccompanied by corrosion or accompanied by relatively little corrosion of hard alloy bearings. This contrasts with excessive corrosion of similar bearings when prior art soaps, such as calcium stearate and calcium naphthenate, are used. Also, used oil inspections (such as increase in viscosity, increase in neutralization number, and increase in naphtha insoluble matter in the used oil) are benefited by the presence of small amounts of the substituted metal alkyl carboxylates of the invention, or at least are not as adversely affected as the commoner soaps and unsubstituted metal alkyl carboxylates. Moreover, the metal alkyl carboxylates of the invention render oils more stable toward oxidation than the base oils.

The following specific examples will show how a number of properties of hydrocarbon oils are 10 benefited by, and will provide a comparison for 20 judging the relative utility of, the substituted metal alkyl carboxylates of the invention.

#### EXAMPLE I

25 A base oil (an SAE 30 blend of 70% Western acid treated naphthenic base oil and 30% Western paraffinic base oil) was tested, with and without the presence of metal alkyl carboxylate additives, to determine its corrosiveness to various alloys of the type used in bearings of internal combustion engines. The "Strip Corrosion Test" was employed in these determinations, this test being as follows:

Thin sheets of the indicated bearing metals 30 were cut into strips (copper-lead,  $\frac{1}{16}$ " x  $1\frac{3}{4}$ " x  $\frac{3}{32}$ "; cadmium-silver,  $\frac{1}{2}$ " x  $1\frac{3}{8}$ " x  $\frac{1}{16}$ "'), and these strips were immersed in the exemplified oils carried in 2" x 20" glass test tubes; these test tubes were carried in an oil bath maintained at 40  $300^{\circ}\text{F.} \pm 1^{\circ}\text{F.}$  Each test tube contained approximately 300 cc. of oil, and air was bubbled through each tube at the rate of 10 liters per hour. At the end of each of three 24-hour periods, the strips were removed from the oils, washed with petroleum ether and carefully wiped with a soft cotton cloth; weight losses of the strips were measured in connection with the weight of each individual strip. The duration of the tests was 72 hours, and the weight losses tabulated below are those found at the end of each 45 24-hour period.

The increase in viscosity of the oil, the neutralization number of the oil at the conclusion 50 of each test, and the amount of naphtha insoluble matter at the conclusion of each test, were also measured. The results of the tests are set forth in Table I below, the additives referred to having been used in the amount of 0.5% by weight based on the oil:

Table I

| Oil                   | Additive                       | Cu-Pb strip |         |         | Cd-Ag strip |         |         | Fresh oil viscosity |         | Used oil viscosity |         | Neutralization number | ASTM naphtha insolubles |
|-----------------------|--------------------------------|-------------|---------|---------|-------------|---------|---------|---------------------|---------|--------------------|---------|-----------------------|-------------------------|
|                       |                                | 24 hrs.     | 48 hrs. | 72 hrs. | 24 hrs.     | 48 hrs. | 72 hrs. | 100° F.             | 210° F. | 100° F.            | 210° F. |                       |                         |
| Western SAE 30 blend. | None                           | 0.8         | 1.6     | 5.5     | 0.0         | 0.0     | 0.0     | 632                 | 57.0    | 1041               | 66.6    | 2.00                  | 109                     |
| Do.                   | Ca butyrate                    | 3.9         | 13.3    | 37.4    | 0.0         | 15.5    | 45.8    | 628                 | 57.1    | 1442               | 76.6    | 4.97                  |                         |
| Do.                   | Ca 2-ethyl butyrate            | 2.5         | 44.0    | 117.0   | 0.0         | 17.0    | 47.1    | 632                 | 57.0    | 1442               | 76.6    | 4.97                  |                         |
| Do.                   | Ca laurate                     | 14.2        | 67.2    | 97.9    | 12.4        | 16.3    | 15.7    | 630                 | 57.3    | 1148               | 70.1    | 4.49                  | 143                     |
| Do.                   | Ca palmitate                   | 47.3        | 125.0   | 166.4   | 9.5         | 38.2    | 90.2    | 632                 | 57.0    | 1361               | 75.5    | 3.07                  | 221                     |
| Do.                   | Ca stearate                    | 84.4        | 152.5   | 208.1   | 0.6         | 34.8    | 82.0    | 633                 | 57.5    | 1340               | 75.0    | 4.02                  | 248                     |
| Do.                   | Ba beta-phosphonatoisobutyrate | +0.4        | +0.8    | +0.5    | 0.1         | 0.2     | 0.3     | 634                 | 56.0    | 844                | 62.4    | 0.44                  | 26                      |
| Do.                   | Ba thiosulfatoacetate          | 0.0         | 0.1     | 0.3     | 0.0         | 0.0     | 0.0     | 630                 | 57.0    | 847                | 62.6    | 1.05                  | 14                      |
| Do.                   | Ca silicatotetraacetate        | 1.4         | 1.6     | 1.4     | +0.2        | +0.2    | +0.4    | 631                 | 57.0    | 1216               | 72.1    | 4.05                  | 218                     |

## EXAMPLE II

Oil was placed in a beaker in contact with air, maintained at a given temperature, and protected against drafts until darkening due to oxidation had occurred. A sample of the original oil was placed in a glass cell 50 mm. square by 7 mm. thick, and an equal sample of the exposed oil was placed in a second similar glass cell. The glass cells were placed equidistant from an electric light. The light that passed through each glass cell was caused to impinge on a photoelectric cell. The two photoelectric cells were mounted in two arms of a Wheatstone bridge. The difference in light transmissions, caused by the different colors of the oils, was thus registered on the Wheatstone bridge. The readings of the bridge were calibrated against the standard ASTM color numbers, and from this the readings of the bridge could be converted into ASTM color numbers (Method D155-34T).

A base oil (Western paraffinic SAE 30) and the same base oil plus 0.5% by weight of inhibitor were tested, substituted metal alkyl carboxylates being used as the inhibitor. The results are set forth in Table II below:

Table II

| Base oil                   | Additive                             | Temperature | ASTM color increase |
|----------------------------|--------------------------------------|-------------|---------------------|
| Western paraffinic SAE 30. | None.....                            | °F. 356     | 8                   |
| Do.....                    | Ba beta-phosphonato-isobutyrate..... | 356         | 5                   |
| Do.....                    | Ba thiosulfatoacetate.....           | 357         | 6½                  |

## EXAMPLE III

The base oil employed was a Western SAE 30 blend (70% Western acid treated naphthenic and 30% Western paraffinic). The additives were calcium alpha-cetylmalonate, calcium alpha-tetradecenyl succinate, calcium alpha-eicosenylsuccinate, and calcium alpha-eicosyltartrate, these additives having the following structural formulae:



Calcium alpha-cetyl-malonate



Calcium alpha-eicosenyl-succinate



Calcium alpha-tetradecenyl-succinate



Calcium alpha-eicosyl-tartrate

5

10 In the formulae,  $\text{R}_1$  represents the normal cetyl ( $\text{C}_{16}\text{H}_{33}$ ) group,  $\text{R}_2$  represents an alkyl group containing, on the average, 12 carbon atoms,  $\text{R}_3$  represents an alkyl group containing, on the average, 18 carbon atoms, and  $\text{R}_4$  represents the group  $\text{C}_{20}\text{H}_{41}$ .

15 The base oil, and the base oil plus the above compounding agents, were submitted to various tests, as follows:

Color stability.—The Deep Rock method was used, in which a 50 gram sample of oil is held 20 in a glass container at 300° F. for 6 hours and at the end of this time the oil was cooled and its color measured and the color increase (ASTM Method D155-34T) over that of the original oil is noted.

25 Oxygen absorption.—The "Oxidator test" described in Industrial and Engineering Chemistry, vol. 28, page 26 (1936) was used. A temperature of 340° F. was used and the results are reported in cubic centimeters of oxygen absorbed 30 per 100 grams of oil.

Corrosion.—The Strip corrosion test of Example 1 was employed.

35 Engine test.—A single cylinder Lauson gasoline spark-ignition engine,  $2\frac{1}{8}$  inch bore and  $2\frac{1}{2}$  inch stroke, loaded with an induction generator, was operated under extremely severe conditions, designed to develop fully the tendency of the crankcase lubricant to deteriorate with gum formation 40 and piston ring sticking: operation was at 1600 revolutions per minute; engine jacket temperature was maintained at 375° F.; crankcase oil temperature was maintained at 220° F.; at periods of 15 hours the operations were interrupted and 45 the condition of the piston rings determined.

Wear.—The Weeks wear testing machine was used. In the operation of this machine a  $\frac{1}{2}$  inch steel ball is pressed against a  $1\frac{1}{8}$  inch steel cylinder which is rotated at 600 revolutions per minute and which dips into the oil being tested. The test lasts 16 hours and the body of the oil is held at 300° F. The results are reported in inches of wear  $\times 10^5$ , as measured on the cylinder.

55 Film strength.—The film strength was measured by the use of the Timken machine as described in the S. A. E. Journal, vol. 28, page 53 (1928), and the results are reported in pounds pressure at failure.

60 During some of the above tests certain other properties were measured, such as viscosity, neutralization number, etc., and the measurements are recorded along with the results of the principal tests.

65 The various test results are recorded in Tables III and IV below. The calcium alpha-cetylmalonate and calcium alpha-eicosenylsuccinate were used in all the tests in the amounts of 0.5% and 0.34%, respectively, by weight based on the oil. In some tests the calcium alpha-tetradecenyl succinate was used in the amount of 0.5% by weight based on the oil, but in others it was used 70 in lesser amounts as indicated in parentheses in

75 the tables below.

Table III

| Base oil              | Additive                               | Color stability (ASTM color increase) | Oxygen absorption (cc. oxygen in 2 hrs.) | Strip corrosion |           |         |             |         |         |                        |         |                       |                          |      |    |
|-----------------------|----------------------------------------|---------------------------------------|------------------------------------------|-----------------|-----------|---------|-------------|---------|---------|------------------------|---------|-----------------------|--------------------------|------|----|
|                       |                                        |                                       |                                          | Cu-Pb strip     |           |         | Cd-Ag strip |         |         | Inspection at 72 hours |         |                       |                          |      |    |
|                       |                                        |                                       |                                          | 24 hrs.         | 48 hrs.   | 72 hrs. | 24 hrs.     | 48 hrs. | 72 hrs. | 100° F.                | 210° F. | Neutralization number | Naphtha insoluble matter |      |    |
| Western SAE 30 blend. | Nil.                                   | 6                                     | 200                                      | 0.7             | 4.7       | 13.9    | 0.1         | 0.2     | 0.4     | 477                    | 11.6    | 2.80                  | 388                      |      |    |
|                       | 0.5% Ca alpha-cetyl-malonate.          |                                       |                                          | 95              | 0.9       | 6.0     | 0.8         | 0.2     | 0.4     | 0.3                    | 220     | 7.0                   | 1.21                     | 29   |    |
|                       | 0.5% Ca alpha-tetra-decenyldsuccinate. |                                       |                                          | 1-(0.18%)       | 30(0.18%) | 0.8     | 1.1         | 1.1     | 0.2     | 0.4                    | 0.3     | 216                   | 6.7                      | 1.33 | 16 |
|                       | 0.34% Ca alpha-eicosenylsuccinate.     |                                       |                                          | ½               | 50        | 0.6     | 1.1         | 1.6     | 0.0     | 0.1                    | 0.1     | 197                   | 6.6                      | 0.68 | 16 |
|                       | 0.63% Ca alpha-eicosyltartrate.        |                                       |                                          | 1-              | 105       | 3.8     | 4.9         | 5.0     | 1.0     | 1.2                    | 0.9     | 296                   | 9.4                      | 1.20 | 62 |

Table IV

| Base oil              | Additive                               | Engine test                  |                                | Weeks wear test, inches wear $\times 10^4$ in 16 hours at 300° F. | Timken film strength, pounds at failure |
|-----------------------|----------------------------------------|------------------------------|--------------------------------|-------------------------------------------------------------------|-----------------------------------------|
|                       |                                        | Hours to cause ring sticking | Relative ring slot cleanliness |                                                                   |                                         |
| Western SAE 30 blend. | Nil.                                   | 30                           | Poor                           | 288                                                               | 120                                     |
|                       | 0.5% Ca alpha-cetyl-malonate.          |                              | Fair                           | 143                                                               | 160                                     |
|                       | 0.5% Ca alpha-tetra-decenyldsuccinate. |                              | Fair+                          | 163(0.2%)                                                         | 120(0.2%)                               |
|                       | 0.34% Ca alpha-eicosenylsuccinate.     |                              | Good                           | 106                                                               | 220                                     |
| Do.                   | 0.63% Ca alpha-eicosyltartrate.        | 60+                          | Fair+                          |                                                                   |                                         |

The substituted metal alkyl carboxylates of the invention may be advantageously added to any hydrocarbon oil or lubricating oil, such as the more viscous distillates and residues from petroleum oil, viscous olefin polymers, and viscous oils derived from oxides of carbon or other forms of carbon by hydrogenation, and they may be added with advantage to any of the newer synthetic lubricants, such as amyl naphthalene. The additives of our invention may be used in viscous hydrocarbon oils ranging in viscosity from about 60 SSU or lower at 100° F. to 160 SSU or higher at 210° F. The metal alkyl carboxylates may be used, in the finished oil, in amounts ranging from 0.1% or less to 10% or more by weight based on the finished oil, but preferably it is used in amounts of about 0.1 to 5%, usually 0.5 to 2%. Concentrates may be prepared containing more than 10% and up to 50% or more of the metal alkyl carboxylate of the invention, alone or together with another additive or other additives, and the concentrate may be diluted with more oil when it is desired to produce the finished oil.

The substituted metal alkyl carboxylates of the invention, as is clear from the examples, are multifunctional in character, and an oil containing one or more of the additives of this invention is improved in several respects. However, the additives of the invention may be advantageously combined in hydrocarbon oils with one or more other additives, such as other antioxidants or corrosion inhibitors, other detergents or anti-ring sticking agents, pour point inhibitors, viscosity and viscosity index improvement agents, oiliness, wear, and film strength agents, etc. Specifically, the additives of this invention may be used in mineral or hydrocarbon oils in combination with any one or more of the following:

(1) Unsubstituted or corrosive carboxylate salts such as the calcium, barium and aluminum

salts of lauric, palmitic, stearic, arachidic, naphthenic, phenyl stearic, benzal stearic, dihydroabietic, oleic, linoleic and alkylated aromatic acids; also various polar substituted metal carboxylates, such as metal salts of chloro stearic, hydroxy stearic, lauric, cetyl hydroxybenzoic, mercaptostearic, cetyl tartaric, cetyl cystine and dodecyl amino benzoic acids.

(2) Metal phenates such as the calcium, barium and aluminum salts of cetylphenol, cetyl chlorophenol and cetylthiophenol.

(3) Metal salts of organo-substituted oxy- and thio-acids of phosphorus, such as calcium cetyl phosphate, aluminum lauryl phosphate and calcium cetyl phenyl phosphate.

(4) Carboxylate esters having an alkyl hydroxy substituent (an hydroxy substituent attached to an alkyl carbon atom) near a carbonyl group of the ester, such as the methyl, ethyl, propyl, butyl, amyl, hexyl, heptyl, octyl, nonyl, lauryl, dodecyl, tetradecyl, cetyl and octadecyl esters of alpha, beta or gamma hydroxy propionic acid, and the corresponding esters of alpha, beta or gamma hydroxy butyric, valeric, caproic, enanthic, caprylic, capric, lauric, myristic, palmitic, stearic, and arachidic acids, as well as the corresponding esters of tartaric, tartaric and citric acids.

The structural formulae and preparation of typical additives capable of use in accordance with this invention are given below:

#### Barium thiosulfatoacetate

The structural formula of this substance is as follows:



19 grams of chloro acetic acid are dissolved in 100 cc. of water and the solution is neutralized with a saturated solution of 10.6 grams of sodium

carbonate. 50.3 grams of sodium thiosulfate pentahydrate are added to the neutralized solution and the solution is evaporated to about one-half of its original volume. The barium salt is then precipitated by adding barium chloride and is filtered off and dried.

*Calcium silicatotetraacetate*

The structural formula of this substance is as follows:



19.0 grams of calcium glycolate are suspended in 150 cc. of benzene and an excess of silicon tetrachloride in benzene solution is added. The salt changes from a powder to a viscous mass. The benzene is poured off and the residue washed with benzene. It is then dried and most of the hydrogen chloride removed by heating to 250° F. under a vacuum of 5 millimeters of mercury for two hours.

*Barium beta-phosphonato-isobutyrate*

The structural formula of this substance is as follows:



500 grams of  $\text{PCl}_3$  are mixed in a 2 liter flask with 800 cc. of dry alcohol-free acetone. 80 grams of aluminum chloride are added in small portions. After the rapid evolution of  $\text{HCl}$  has subsided the flask is heated on a water bath to remove additional  $\text{HCl}$ . Diacetone phosphorus chloride is thus formed. It is hydrolyzed by adding it to water. The resulting impure diacetone phosphinic acid is recovered by evaporating off the water. It is purified by dissolving it in alcohol and precipitating the ammonium salt with ammonia. This ammonium salt is washed with alcohol, dissolved in water and filtered. The acid is obtained by acidification with  $\text{HCl}$  followed by evaporation. The solid residue is extracted with alcohol, filtered and evaporated to dryness. The purified diacetone phosphonic acid is oxidized with nitric acid and then with fuming nitric acid. The excess fuming nitric acid is removed by heating on a water bath. The impure beta-phosphonato butyric acid is dissolved in water and barium hydroxide is added until it is strongly alkaline. This solution is heated to boiling and filtered. The filtrate is discarded since the barium salt of the desired acid is only slightly soluble in hot water, while impurities dissolve. The residue remaining on the filter is extracted with cold water and the extract is evaporated to dryness.

*Calcium alpha-cetylmalonate*

The structural formula of this substance is given in Example 3 above.

Sodium ethylate is produced by treating 100 cc. of absolute alcohol with 12 grams of sodium. Sodium diethyl malonate is then precipitated by adding 80 grams of diethyl malonate to the sodium ethylate. Diethyl alpha-cetylmalonate is then formed by adding 190 grams of cetyl iodide to the above sodium diethyl malonate and heating the mixture at 212° F. Sodium iodide is removed by washing with water. Potassium alpha-cetylmalonate is then made by hydrolyzing the diethyl alpha-cetylmalonate with 520 cc. of a 10% KOH solution employing a temperature of 212° F. for 24 hours. The potassium salt is salted out from the aqueous solution,

washed, dried, and extracted with ethyl ether to remove excess cetyl iodide. The desired calcium alpha-cetylmalonate is then prepared by suspending 100 grams of potassium salt in a 50-50 alcohol-water mixture, heating the mixture to 190° F. and adding excess calcium chloride solution. The precipitate is washed and dried, yielding the desired calcium alpha-cetylmalonate.

*Calcium alpha-tetradecenylsuccinate*

The structural formula of this substance is given in Example 3 above.

An olefinic polymer of average chain length  $\text{C}_{14}$  produced as a high boiling residue in the production of gasoline by polymerization of olefins is mixed in 25% excess over molecular proportion with maleic anhydride and the mixture is heated in an iron pressure vessel, without agitation, at 400-450° F. for 4 to 6 hours. The pressure developed does not exceed 110 pounds per square inch. The product, tetradecenylsuccinic anhydride, is distilled under vacuum to remove unreacted polymers and maleic anhydride. A neutralization number of the tetradecenyl succinic anhydride is then taken to determine the amount of water theoretically required for hydration. The theoretical amount of water is added and the anhydride is digested under reflux for 1 hour at 195° F., thus forming tetradecenylsuccinic acid. A neutralization number of the acid is taken to determine the amount of potassium hydroxide required for making the potassium salt. The tetradecenylsuccinic acid is neutralized by heating at 180° F. for 30 minutes with a slight excess of potassium hydroxide in 25% aqueous solution. The desired calcium alpha-tetradecenylsuccinate is prepared by adding an equivalent amount of calcium chloride in 10% solution to the solution of potassium salt as obtained above. The product is obtained as a white, curdy precipitate which is washed free of impurities.

*Calcium alpha-eicosenylsuccinate*

The structural formula of this substance is also given in Example 3 above. It is prepared in exactly the same manner as calcium alpha-tetradecenylsuccinate except that a  $\text{C}_{20}$  olefin polymer is used in place of the  $\text{C}_{14}$  olefin polymer.

We claim:

1. A composition of matter, comprising a major proportion of a hydrocarbon oil and a small amount, not less than about 1% by weight based on finished oil, of a metal alkyl carboxylate, substituted on an alpha, beta or gamma alkyl carbon atom with respect to a metal alkyl carboxylate group by a substituent containing at least one element of the group consisting of metals and metalloids and at least one element of the group consisting of oxygen and sulfur.

2. A composition of matter, comprising a major proportion of an oil of lubricating viscosity and a small amount, not less than about 0.1% by weight based on finished oil, of a metal alkyl carboxylate substituted on an alpha, beta or gamma alkyl carbon atom with respect to a metal alkyl carboxylate group by a substituent containing at least one element selected from the group consisting of metals and metalloids and at least one element from the group consisting of oxygen and sulfur, said substituent being attached to said alkyl carbon atom through one of said elements.

3. The composition of claim 2, wherein said substituent contains a metal and oxygen.
4. The composition of claim 2, wherein said substituent contains a metal and sulfur.
5. The composition of claim 2, wherein said substituent contains a metalloid and oxygen.
6. The composition of claim 2, wherein said metal alkyl carboxylate is an alkaline earth metal carboxylate.
7. A composition of matter, comprising a major proportion of a hydrocarbon oil of lubricating viscosity and a small amount, sufficient to improve the oil, of an oil-soluble polyvalent metal alkyl carboxylate substituted on an alpha, beta or gamma alkyl carbon atom with respect to a metal alkyl carboxylate group by a substituent containing a metal, oxygen and phosphorus.
8. A composition of matter, comprising a major proportion of a hydrocarbon oil of lubricating viscosity and a small amount, sufficient to improve the oil, of an oil-soluble polyvalent metal alkyl carboxylate substituted on an alpha, beta or gamma alkyl carbon atom with respect to a metal alkyl carboxylate group by a substituent containing a metal, sulfur and phosphorus.
9. A composition of matter, comprising a major proportion of a hydrocarbon oil of lubricating viscosity and a small amount, sufficient to improve the oil, of an oil-soluble polyvalent metal alkyl carboxylate substituted on an alpha, beta or gamma alkyl carbon atom with respect to a metal alkyl carboxylate group by a substituent containing a metal, sulfur and oxygen.
10. A composition of matter, comprising a major proportion of a hydrocarbon oil of lubricating viscosity and a small amount, sufficient to improve the oil, of an oil-soluble polyvalent metal alkyl carboxylate substituted on an alpha, beta or gamma alkyl carbon atom with respect to a metal alkyl carboxylate group by a substituent containing boron and oxygen.
11. A petroleum lubricating oil containing about 0.1 to 5% by weight based on finished oil of a polyvalent metal alkyl carboxylate substituted on an alpha, beta or gamma alkyl carbon atom with respect to a metal alkyl carboxylate group by a substituent containing at least one element selected from the group consisting of metals and metalloids and at least one element selected from the group consisting of oxygen and sulfur.
12. The composition of claim 11, wherein said polyvalent metal is an alkaline earth metal.
13. A composition of matter, comprising a concentrated solution in viscous mineral oil of a metal alkyl carboxylate substituted on an alpha, beta or gamma alkyl carbon atom with respect to a metal alkyl carboxylate group by a substituent containing at least one element selected from the group consisting of metals and metalloids and at least one element selected from the group consisting of oxygen and sulfur.
14. A lubricant comprising a mineral oil of lubricating viscosity and about 0.1 to 5% by weight based on the lubricant of a polyvalent metal salt of an aliphatic carboxylic acid substituted on an aliphatic carbon atom alpha, beta or gamma to a metal alkyl carboxylate group by a metallo mercapto group.
15. A lubricant comprising a mineral oil of lubricating viscosity and about 0.1 to 5% by weight based on the lubricant of a polyvalent metal salt of an aliphatic carboxylic acid substituted on an aliphatic carbon atom alpha, beta or gamma to a metal alkyl carboxylate group by a metallo phosphonato group.
16. A lubricant comprising a mineral oil of lubricating viscosity and about 0.1 to 5% by weight based on the lubricant of a polyvalent metal salt of an aliphatic carboxylic acid substituted on an aliphatic carbon atom alpha, beta or gamma to a metal alkyl carboxylate group by a metallo thiophosphonato group.
17. A petroleum lubricating oil comprising about 0.1 to 5 per cent by weight based on finished oil of a polyvalent metal salt of a fatty acid containing not less than ten carbon atoms and substituted on an alpha, beta or gamma carbon atom with respect to the metal carboxylate group by a substituent containing at least one element selected from the group consisting of metals and metalloids and at least one element selected from the group consisting of oxygen and sulfur, said substituent being attached to said alkyl carbon atom through one of said elements.
18. A petroleum lubricating oil comprising a small amount each of a metal salt of a phenol and a metal alkyl carboxylate substituted on an alpha, beta or gamma alkyl carbon atom by a substituent containing at least one element selected from the group consisting of metals and metalloids and at least one element selected from the group consisting of oxygen and sulfur, said substituent being attached to said alkyl carbon atom through one of said elements, said salt of phenol and said carboxylate being present in respective amounts and in relative proportions sufficient to provide a lubricant of enhanced detergency and low corrosivity in the crankcase of an internal combustion engine.
19. The oil of claim 18 wherein said metal salt of phenol and said metal alkyl carboxylate are oil-soluble, polyvalent metal salts.

BRUCE B. FARRINGTON.  
JAMES O. CLAYTON.  
DORR H. ETZLER.